

Patented May 7, 1929.

1,712,252

# UNITED STATES PATENT OFFICE.

NARAINA DAS CHOPRA AND FREDERICK JOHN BULLEN, OF WESTMINSTER, LONDON, ENGLAND.

## MANUFACTURE OF ROLLED-STEEL MEMBERS.

No Drawing. Application filed December 10, 1926, Serial No. 154,028, and in Great Britain January 2, 1926.

This invention relates to the manufacture of rolled steel members and for the sake of convenience will be described by reference to the manufacture of steel rails as typifying 5 rolled steel members. It is to be understood, however, that the invention is not limited to the manufacture of steel rails but is applicable to the manufacture of any form of rolled steel member.

10 In the ordinary manufacture of steel rails there occurs a zonic heterogeneity of structure which may be said to be characterized by the presence of three zones, namely, a central zone of pearlitic nature, an outer zone of soft 15 decarburized steel, and an intermediate zone of high-carbon steel. This zoning of structure is generally accompanied by a state of internal instability, and has been found to be mainly responsible for the faults commonly 20 experienced in rails, of corrugation and excessive wear and tear in use.

It is known to be possible to remove from steel defects of the kind referred to above by annealing, i. e. by a treatment comprising 25 heating the steel to a high temperature and thereafter allowing the metal to cool slowly. Such treatment, however, is generally associated with the disadvantage of producing softening of the steel; it does not eliminate 30 from the structure of the steel the aforesaid zonic heterogeneity, and, further, it leads to the formation of scale, with an accompanying loss of steel by weight.

According to the present invention, a process 35 of manufacture of rolled steel members is characterized in this, that the hot member from which the rail is being formed is submitted one or more times during the formation of the rail, for example, between successive rolling operations, to a treatment which involves a temperature drop to a point below the lowest change-point of the metal and following this a reheating of the member to the appropriate temperature for the succeeding 40 forming operation. By "lowest change point", we mean the lowest critical point, and have designated this point in some of the claims as the "Ar change point", in accordance with common practice.

50 The effect of heat-treatment according to the invention is to remove the aforesaid structural defects, or, according to circumstances, materially to reduce them; and where such defects are not wholly removed the hot member 55 may be subjected after completion of its

forming operations, to the final heat-treatment process set forth in the specification of our British Letters Patent, No. 271,529 of 1927. That is to say, the hot completely-formed member may be cooled to a temperature below the lowest change-point of the metal, then heated to a temperature above (e. g. 50° above) the highest change-point, cooled gradually to a temperature somewhat below (e. g. 50° C. below) the lowest change-point, and finally allowed more rapidly to cool, e. g. by allowing the member to cool spontaneously in the atmosphere.

We have found it preferable, and it is a further feature of this invention, to conduct 70 the heat treatment characterizing this invention in the presence of an oxidation inhibitor by which is meant a solid material which is non-fusible at the temperature employed in the heat treatment and the action of which, 75 through chemical affinity of the material towards the deleterious furnace gases, is to protect the metal from oxidation or substantially to reduce the degree thereof. Examples of 80 oxidation inhibitors are alkaline earth oxides, such as lime; infusible readily-oxidizable materials in a condition to present to the gases a large surface relatively to the area of the exposed surface of the member under heat treatment, for example, shavings or turnings of an 85 oxidizable metal such as steel; and carbonaceous material, such as an exhausted carburizing mixture, boiler-ash or producer-ash, containing an adequate proportion (for example, at least 10 per cent) of combustible carbon.

90 By an exhausted carburizing mixture is meant a carburizing mixture which has been used to such an extent as to render it unsuitable for further use in carburizing. A suitable carburizing mixture which, when exhausted, has been found to be utilizable according to the present invention consists of three parts of powdered beech charcoal and two parts each of powdered horn charcoal and powdered animal charcoal. The boiler-ash 95 or producer-ash may be of the type which usually contains from 5 to 15 per cent of carbon.

100 The use in heat-treatment of steel of a mixture of alkaline earth oxide and an appropriate carbonaceous material carrying free carbon such as an exhausted carburizing reagent, forms the subject of our British Letters Patent No. 271,606 of 1927, and is claimed herein only in conjunction with the special heat- 110

treatment which characterizes the present invention.

The beneficial effects of the process according to the present invention are generally found to be influenced by the degree of cooling to which the member is subjected between the forming operations; and in such cases, where commercial exigencies permit, the cooling may, with advantage, be carried 10 to a degree considerably below the lowest change-point of the metal, and even to atmospheric temperature.

We have frequently found in our work upon steel members that the process of this 15 invention gives specially good results in the case of steel containing a small proportion of a metallic element, such as nickel or cobalt, the presence of which tends to depress the change-points of the steel.

20 According to a further feature of the invention, therefore, the steel member subjected to the aforesaid special heat-treatment is composed of steel containing a small proportion of a metallic change-point depressant, 25 such, for example, as nickel or cobalt.

The proportion necessary of such element is preferably quite small, for example, 1 per cent or less. We have usually found 0.5 per cent to be sufficient. In this connection it 30 will be understood that the advantage in question is secured with steel wherein the nickel or other change-point depressant is present even as an adventitious component.

We have also found that the heat-treatment characteristic of this invention is 35 especially effective in the case of chrome steels; and according to a further feature of the invention the steel member subjected to heat-treatment as above is composed of chrome- 40 steel. We have found that with this particular special metal the advantageous effects of the invention are frequently very marked.

The chrome-steel from which the member is formed may with further advantage be a 45 chrome-steel containing a change-point depressant, such as nickel or cobalt.

Reverting again to the oxidation inhibitors the presence of which as aforesaid is 50 preferable during the heat-treatment which characterizes this invention, the inhibitor may comprise sheets or plates of an oxidizable metal such as iron or steel disposed around the walls of the furnace or beneath the roof thereof or in the gas openings. Alternatively, the steel member to be protected may 55 be enveloped during the heat-treatment in a cage built up of sheets or plates or bars of iron or steel or other readily oxidizable metal.

Again, if an alkaline earth oxide such as 60 lime be employed as the oxidation inhibitor it may be employed in powder form or in aqueous suspension or solution. The manner of applying the oxide may be varied according to circumstances and convenience.

65 If the member under heat-treatment is the

initial hot ingot, or is in the billet stage, or, again, is proceeding through the rolling mills, the oxide may be sprayed or dropped upon the member. On the other hand, if the member is undergoing heat-treatment in a 70 soaking-pit, reheating furnace or other furnace, the member may be placed in a bath of powdered lime or like oxide or a paste of the oxide may be coated upon the member.

In some cases it may be found preferable 75 either as an alternative to the aforesaid forms and modes of application of oxidation inhibitor or in conjunction therewith to line the soaking pit or other furnace with dolomite or furnace slag.

80 Lastly, with regard to the oxidation inhibitors, any two or more of the aforesaid forms may be employed conjointly.

#### Example 1.

85 Two ingots were cast, with the following analyses:—

|            | A.      | B.      |
|------------|---------|---------|
|            | Percent | Percent |
| Carbon     | .563    | .563    |
| Silicon    | .112    | .112    |
| Sulphur    | .033    | .033    |
| Phosphorus | .043    | .043    |
| Manganese  | .80     | .80     |
| Nickel     | —       | .55     |

90 The tapping temperatures were 1530° C. 1520° C.

The teaming temperatures (with one inch nozzle) were 1450° C. 1450° C.

95 Ingot A. was treated and rolled right through, according to the normal practice prevailing in the steel works.

Ingot B. was treated and rolled in accordance with the present invention. The top of the ingot mould was covered during setting with an oxidation protector as aforesaid consisting of an exhausted carburizing mixture. On stripping, the ingot was spread over with the aforesaid oxidation protector. The stripping temperature was 960° C. The ingot was transferred to the soaking pit, the floor of which was covered to a depth of about three inches with a mixture of boiler ash, carrying 105 15.6 per cent. of combustible carbon, and lime, in the proportions of 60-40, while sufficient steel turnings to cover, when loosely spread, a surface of at least half an inch along the bed of the pit, were packed therein around the ingot. The top lids of the pits 110 were provided with a mass of steel turnings so suspended from the lids that practically the whole space between the top of the ingot and the roof of the furnace was occupied by the turnings. The ingot was transferred to 115 the cogging mill at 1190° C. The billet passed the saw at a temperature of 940° C. and was then allowed to cool down to 600° C.

120 The cooling down was carried out with the billet covered with an oxidation protector 125 130

similar to that employed in the soaking pits. It was then reheated to 960° C., again in the presence of the oxidation protector, and then subjected to rolling operations to form a rail without any further treatment. It was found that without sacrifice of tensile strength, both the elongation and the reduction of area of the test piece were very materially increased by the special treatment characteristic of this invention as compared with the rail from ingot A.

|          | Max-<br>imum<br>strength. | Elonga-<br>tion on<br>3". | Reduc-<br>tion of<br>area. |
|----------|---------------------------|---------------------------|----------------------------|
|          | Per cent.                 | Per cent.                 |                            |
| Sample A | 53.24                     | 11                        | 16.3                       |
| Sample B | 53.42                     | 18                        | 27.4                       |

The structure of the rail showed itself to be in a homogeneous pearlitic form, and the rail exhibited no sign of a decarburized zone at the surface.

*Example 2.*

The analysis of the steel was as follows:

|            | Per cent. |
|------------|-----------|
| Carbon     | .563      |
| Silicon    | .196      |
| Sulphur    | .023      |
| Phosphorus | .036      |
| Manganese  | .73       |
| Nickel     | .35       |
| Chromium   | .98       |

The operations of pouring, teaming, cogging, and rolling were carried through as in the case of sample B of Example 1.

The billet reached the saw at 920° C., was then cooled down to 650° C. and reheated to 940° C., both cooling and reheating being conducted in the presence of an oxidation protector as in Example 1.

The billet was then subjected to rolling operations to form a rail. The test figures were as follows:

| Maximum<br>strength. | Elongation. | Reduction<br>of area. | Brinell. |
|----------------------|-------------|-----------------------|----------|
| 51.36                | 20.0        | 41.5                  | 3.7/269  |

In this case the increase of elongation and reduction of area of test piece without loss of tensile strength was even more marked than in the case of the sample B product of Example 1.

The corresponding figures for a rail produced by ordinary steel works practice and of the same analysis were:

| Maximum<br>strength. | Elongation. | Reduction<br>of area. | Brinell. |
|----------------------|-------------|-----------------------|----------|
| 49.06                | 1.0         | 2.0                   | 3.6/286  |

It is to be understood, in conclusion, that the special heat-treatment which broadly

characterizes this invention, namely, the treatment which comprises cooling the hot partially-formed member to a temperature below the lowest change-point of the metal, and following this a reheating of the member to the appropriate temperature for the succeeding forming operation, may be applied to the member at any time during its formation, from the billet-stage onwards.

We claim:

1. In the manufacture of rolled steel members, interposing, during the process of formation of the member, a heat-treatment which comprises cooling the hot member through the Ar change-points of the steel and so thereafter re-heating to the temperature requisite to further formation, the re-heating operation being effected by direct contact with hot furnace gases which have been rendered substantially innocuous towards the steel as regards their oxidizing and decarburizing capacity by treatment with both an alkaline earth oxide and a substantially non-carburizing carbon-carrying material as herein defined.

2. In the manufacture of rolled steel members, interposing, during the process of formation of the member, a heat treatment which comprises cooling the hot member through the Ar change-points of the steel in the presence of material capable of inhibiting oxidation and thereafter reheating to the temperature requisite to further formation by direct contact with furnace gases which have been rendered substantially innocuous towards the steel as regards their oxidizing and decarburizing capacity by treatment with both an alkaline earth oxide and a substantially non-carburizing carbon-carrying material as herein defined.

3. A process of manufacture of rolled steel members according to claim 1, wherein the relative amounts of the reagents are such that the quantity of oxide is equivalent to from 10% to 50% by weight of the combined quantities of oxide and carbon-carrying material and the carbon content of the carbon-carrying material is such that the quantity of free carbon present is equivalent to from 4% to 20% by weight of the aforesaid combined quantities.

4. A process of manufacture of rolled steel members according to claim 1, wherein the reheating operation is effected in the presence of a false increase of area of oxidizable material provided by a mass of infusible readily oxidizable material substantially as and for the purpose set forth.

5. In the manufacture of rolled steel members, interposing, during the process of formation of the member, a heat-treatment which comprises cooling the hot member through the Ar change-points of the steel and thereafter reheating to the temperature requisite to further formation, the reheating

operation being effected by direct contact with hot furnace gases which have been rendered substantially innocuous towards the steel as regards their oxidizing and decarburizing capacity by treatment with both lime and a substantially non-carburizing carbon-carrying material as herein defined, the relative amounts of lime and carbon-carrying material being such that the quantity of lime employed is equivalent to from 10% to 50% by weight of the combined quantities of lime and carbon-carrying material and the carbon content of the carbon-carrying material is such that the quantity of free carbon present is equivalent to from 4% to 20% by weight of the aforesaid combined quantities.

6. A process of manufacture of rolled steel members according to claim 5, wherein the reheating step is effected in the presence of a false increase of area of oxidizable material provided by a mass of infusible readily oxidizable material.

7. A process of manufacture of rolled steel members according to claim 5, wherein the cooling step is effected in the presence of both lime and a substantially non-carburizing carbon-carrying material as herein defined, the relative amounts of lime and carbon-carrying material being such that the quantity of lime employed is equivalent to from 10% to 50% by weight of the combined quantities of lime and carbon-carrying material and the carbon content of the carbon-carrying material is such that the quantity of free carbon present is equivalent to from 4% to 20% by weight of the aforesaid combined quantities.

8. In the manufacture of rolled steel members, interposing, during the process of formation of the member, a heat-treatment which comprises cooling the hot member through the Ar change-points of the steel in the presence of material capable of inhibiting

oxidation of the steel, and thereafter reheat-  
ing the member to the temperature requisite 45  
for further formation by direct contact with  
hot furnace gases in a furnace containing a  
mixture of lime and substantially non-car-  
burizing carbon-carrying material as herein  
defined, the relative amounts of the lime and 50  
carbon-carrying material being such that the  
quantity of lime employed is equivalent to  
from 10% to 50% by weight of the combined  
quantities of lime and carbon-carrying mate-  
rial and the carbon content of the carbon- 55  
carrying material is such that the quantity  
of free carbon present is equivalent to from  
4% to 20% by weight of the aforesaid com-  
bined quantities.

9. A process of manufacture of rolled steel 60  
members according to claim 8, wherein the  
furnace contains also a mass of infusible  
readily oxidizable material providing a false  
increase of oxidizable surface area in ex-  
posure in the furnace to the furnace gases. 65

10. A process of manufacture of rolled steel  
members according to claim 8, wherein the  
carbon-carrying material is a carburizing  
mixture which has been used to such an extent  
as to have become substantially exhausted 70  
of its carburizing capacity.

11. A process of manufacture of rolled steel  
members according to claim 8, wherein the  
steel of which the member is composed con-  
tains a small proportion of a change-point 75  
depressant.

12. A process of manufacture of rolled steel  
members according to claim 8, wherein the  
steel of which the member is composed is  
chrome-steel containing a small proportion 80  
of a change-point depressant.

In testimony whereof we have signed our  
names to this specification.

NARAINA DAS CHOPRA.  
FREDERICK JOHN BULLEN.